

# United States Patent

111 3,583,193

[72] Inventor Kanichi Kishikawa  
Fukuoka, Japan  
[21] Appl. No 782,174  
[22] Filed Dec. 9, 1968  
[45] Patented June 8, 1971  
[73] Assignee Nippon Steel Corporation  
Tokyo, Japan  
[32] Priority Dec. 16, 1967  
[33] Japan  
[31] 42/80439

[54] ROLLING METHOD AND APPARATUS FOR  
PRODUCING H-SHAPED STEEL PRODUCTS  
HAVING FLANGES OF DIFFERENT THICKNESSES  
AND SIMILARLY SHAPED STEEL PRODUCTS  
3 Claims, 6 Drawing Figs.

[52] U.S. Cl..... 72/225  
[51] Int. Cl..... B21b 13/10

[50] Field of Search ..... 72/225, 366

[56] References Cited  
UNITED STATES PATENTS  
431,623 7/1890 Sack ..... 72/225  
657,964 9/1900 Seaman ..... 72/225X  
3,342,053 9/1967 Stammbach ..... 72/225X

Primary Examiner—Milton S. Mehr  
Attorney—Wenderoth, Lind and Ponack

**ABSTRACT:** A rolling method and apparatus for producing such shaped products as asymmetrical H-shaped steel products having flanges of different thicknesses by using the universal rolling mill having a pair of vertical rolls, one having greater diameter than the other, thereby making equal or nearly equal the projected lengths of biting contact of these vertical rolls on the rolled material.



PATENTED JUN. 8 1971

3,583,193

SHEET 1 OF 3

FIG. 1A



FIG. 1B



FIG. 2  
PRIOR ART



KANICHI KISHIKAWA,  
INVENTOR

BY, *Wendell L. French*

ATTORNEYS

PATENTED JUN 8 1971

3,583,193

SHEET 2 OF 3

FIG. 3



FIG. 4



KANICHI KISHIKAWA,

INVENTOR

BY, *Wendworth, Sida & Ponack*

ATTORNEY'S

PATENTED JUN 8 1971

3,583,193

SHEET 3 OF 3

FIG. 5



KANICHI KISHIKAWA,  
INVENTOR

BY, *Wendt, Lind, Ponack*

ATTORNEY S

**ROLLING METHOD AND APPARATUS FOR PRODUCING H-SHAPED STEEL PRODUCTS HAVING FLANGES OF DIFFERENT THICKNESSES AND SIMILARLY SHAPED STEEL PRODUCTS**

**BACKGROUND OF THE INVENTION**

1. Field of the Invention

The present invention relates to a rolling method and apparatus for producing H-shaped steel products having flanges of different thicknesses, rails, etc. by using a universal rolling mill.

2. Description of the Prior Art

It has long been well known that, in general, the greater the size of the parts of H-shaped steel products having flanges on both sides of a web or other similarly shaped products such as rails, the more difficult is rolling by conventional roll passes, using horizontal rolls only. The invention of the universal rolling mill using vertical rolls in addition to horizontal rolls, has nearly solved the above problem. Not only has the rolling process using the universal rolling mill solved the problem of the size limit of the flanges of shaped steel products, but also it is effective in such rolling operations concentratedly carried out on the head of such steel products as rails which require heavy forging.

However, the universal rolling mill is not completely free from problems. When producing H-shaped steel products having flanges of different thicknesses, such as rails or the like, with the ordinary type of universal rolling mill having vertical rolls of the same diameter, the rolled material tends to bend and twist while rolled, causing inaccurate size-stability of the product or, at the worst, making it impossible to finish rolling, for such reasons as the difference in stretching rate of the two flanges and the difference in horizontal pressure of the two vertical rolls. That is to say, it is impossible for the universal rolling mill having vertical rolls of the same diameter to roll the material to produce such products having flanges of different thicknesses such as H-shaped steel products and rails.

**SUMMARY OF THE INVENTION**

An object of the present invention is to provide a rolling method and apparatus for rolling the material by using the universal rolling mill with the vertical rolls having been so arranged as to have different diameters, into such shaped products as H-shaped steel products having flanges of different thicknesses, such as rails.

Another object of the present invention is to provide a universal rolling mill capable of rolling the material easily and accurately into such shaped products as H-shaped steel products and rails, which has heretofore been impossible with the conventional universal rolling mill.

In order to achieve the above objects of the present invention, in the production of such shaped products as H-shaped steel products having flanges of different thicknesses and rails by using the universal rolling mill, a pair of the vertical rolls of the universal rolling mill are so constructed that the diameter of one of them is made smaller than that of the other in correspondence with the difference in thickness of the flanges of the to-be-made product, thereby making equal or nearly equal the projected lengths of biting contact of these vertical rolls on the rolled material.

**BRIEF DESCRIPTION OF THE DRAWINGS**

FIG. 1 shows an example of shaped steel products to be rolled by the method and apparatus of the present invention; FIG. 1 (A) and (B) show steel products shaped like rails and H-shaped steel products, respectively.

FIG. 2 is the longitudinal section of the conventional mill when rolling the material into a H-shaped steel product having flanges of different thicknesses to show the relation between the vertical roll and the material.

FIG. 3 is schematic diagram of the vertical roll of the conventional mill when operating, to show the relation with the material in comparison with the relation when operating the mill of the present invention.

5 FIG. 4 is another example similar to that shown in FIG. 3.

FIG. 5 is the longitudinal section of the rolling apparatus of the present invention when operated by the method of the present invention to produce a rail, and showing the relation between the vertical roll and the material.

10

**DESCRIPTION OF THE PREFERRED EMBODIMENT**

The following is explanation of a preferred embodiment of the present invention, in comparison with which is attached 15 the practice of the conventional method to make the explanation more understandable.

It is difficult for the conventional type of the universal rolling mill having vertical rolls of same diameter to roll the material into such shaped steel products having flanges of different thicknesses as H-shaped steel products.

The above difficulty is due mainly to the difference in stretching rate between the two flanges, and also due to the difference in horizontal pressure acting on the two vertical rolls. With reference to FIG. 2 and FIG. 3, horizontal pressure acting on the vertical rolls of the universal rolling mill may be generalized, as follows:

$$\text{Horizontal pressure } P = f B e$$

30 Where:

*f*: Deformity resistance kg./mm.<sup>2</sup>

*B*: Height of flange of the rolled material

*e*: Projected length of biting contact;  $\sqrt{2R\Delta h}$

(*R*: Diameter of the vertical roll)

(*h*: Reduction)

If a final product having the thinner flange 2.5 times higher than the thicker flange and the thicker flange twice thicker than the thinner flange is to be produced with a universal rolling mill having vertical rolls of the same diameter, the

40 horizontal pressure acting on the vertical roll having the thicker flange *P<sub>h</sub>* and that acting on the vertical roll having the thinner flange *P<sub>f</sub>* are formulated, as follows:

$$P_h = B_h e_h = f B_h \sqrt{2R\Delta h_h}$$

$$P_f = B_f e_f = f B_f \sqrt{2R\Delta h_f}$$

$$\text{Since } B_f = 2.5 B_h \Delta h_f = \Delta h_h / 2,$$

$$\text{so } P_f = 1.57 f B_h \sqrt{2R\Delta h_h}$$

Therefore, *P<sub>h</sub>* < *P<sub>f</sub>*

The imbalance of horizontal pressure acting on the vertical rolls 1 and 2 causes the following problems: The vertical roll 1

55 which is effected by greater vertical pressure tends to push the horizontal rolls 4 and 4' through the thinner flange 6 to the left. As the distance between the vertical rolls 1 and 2 is maintained a predetermined constant, the above sideslip (transverse) of the horizontal rolls 4 and 4' affects the formation of the thicker flange 5 placed between these rolls and the other vertical roll 2. If this is left unadjusted, it will become impossible to obtain products of accurate size. In order to prevent sideslip of the horizontal rolls, prior art device called a "thrust

60 metal" is set on the neck of the horizontal roll in the roll housing. This device, however, is not desirable for such rolling methods as that of the present invention which is accompanied with extremely great horizontal pressure, for the following reasons: The thrust metal is subjected to severe abrasion; the thickness of product is inconstant; it requires time and labor for repairs, hampering smooth rolling operations; and also its complicated structure enhances construction costs.

65 Another difficulty is that the vertical rolls 1 and 2 contact the rolled material at different points, therefore, as shown in

FIG. 3, the line connecting the contact point  $Q_1$  of the thicker flange 5 of the rolled material and the contact point  $Q_2$  of the thinner flange 6 of the rolled material, which is rolled between the vertical rolls 1 and 2 and between the horizontal rolls 4 and 4' and the line connecting the centers  $O_1$  and  $O_2$ , respectively, of the vertical rolls 1 and 2 are not parallel. Therefore, when the rolled material enters between the vertical rolls at a right angle to the axes of the vertical rolls  $O_1$  and  $O_2$ , the contact point  $Q_1$  contacts the rolls earlier than the contact point  $Q_2$ , causing the above mentioned horizontal pressure  $P_h$  to produce a bending moment which bends the rolled material in the direction indicated by arrow 7 until the line connecting the contact points  $Q_1$  and  $Q_2$  becomes parallel with the line connecting the centers  $O_1$  and  $O_2$ . In this case, the rolled material is "rubbed down" by the sidewall of the horizontal rolls 4 and 4', such rub producing scratches on the surface of the rolled material.

For the above-mentioned reasons it is difficult for the ordinary universal rolling mill to produce H-shaped steel products having flanges of different thicknesses.

The above is an explanation of the present invention using an example of rolling a prefigured steel piece which, before being fed into the universal rolling mill, has a size and shape similar to those of the desired final product, that is, the part to become the thicker flange of the final product made thicker than the part to become the thinner flange of the final product. This explanation can also apply to the rolling of a prefigured steel piece having the same thickness for parts to become the flanges of the final product, into a final product having flanges of different thicknesses.

In reference to FIG. 4:

$$P_A = f B_A e_A = f B_A \sqrt{2 R_A \Delta_A}$$

$$P'_W = f B_W e'_W = f B_W \sqrt{2 R_A \Delta_W}$$

If the same size of the final product as mentioned above is intended,

$$\Delta T_W = 2 \Delta T_A, B_W = 2.5 B_A$$

$$\text{So } P'_W = f B_W \sqrt{2 R_A \Delta_A}$$

Therefore,  $P'_W > A$

This means that the line connecting  $Q_3$  and  $Q_4$ , which are the contact points of the rolled material respectively with the vertical rolls 1 and 2 is not parallel with the line connecting the centers  $O_1$  and  $O_2$  of the rolls. Thus, the problems as mentioned above will take place on the side of the opposite roll 2.

The present invention is intended to solve these problems by adjusting the diameter of the vertical rolls for rolling to produce, above all, H-shaped steel products having flanges of different thicknesses or other steel products of a similar shape. The special characteristics of the present invention relating to a rolling method and apparatus for producing such asymmetrical steel products as H-shaped steel products having flanges of different thicknesses with the universal rolling mill, consist in that the diameter of one vertical roll is made greater than that of the other vertical roll, thereby making equal or nearly equal the projected lengths of biting contact of the vertical rolls on the rolled material.

Thus,  $Q_2$  and  $Q_3$  or  $Q_3$  and  $Q_5$  which are the contact points of respective vertical rolls with the rolled material become parallel, and the difference, if any, of horizontal pressure will not cause bending moment on the rolled material, thus making possible rolling without bending. Also, as mentioned below, any difference in horizontal pressure may be directed in a predetermined direction so as to have the vertical roll of smaller diameter on the opposite side of this thrust contact the horizontal roll and thus absorb the side-slip of the horizontal roll, thereby completely solving the problems of conventional rolling.

The following is a concrete explanation of the present invention using FIG. 3 and FIG. 5. In these figures are shown rolls for producing rails from a prefigured steel piece having a part to become the thicker flange of the product thicker than the part to become the thinner flange of the product. First of all, a predetermined distance is maintained between the upper horizontal roll 4 and the lower horizontal roll 4' so as to maintain constant the thickness of web T; and the case 8 housing a pair of the vertical rolls 1 and 3 is placed within the same perpendicular section of said horizontal rolls 4 and 4'. In this case, the diameter of the vertical roll 3 on the side of the head 9 of the rail to be subjected to greater reduction is made smaller than that of the vertical roll 1 on the side of the base 10 of the rail to be subjected to smaller reduction. As shown in FIG. 3, the line connecting the contact points  $Q_2$  and  $Q_5$  respectively of the vertical rolls 1 and 3 with the rolled material is made parallel with the line connecting the centers  $O_2$  and  $O_3$  of the vertical rolls, so as to make equal the projected lengths  $e_h$  and  $e_f$  of biting contact of the rolls on the rolled material.

In practice the rolling schedule is predetermined with relation to the size of the prefigured steel piece and that of the product, and to the number of passes and reduction by respective passes. The diameters of the vertical rolls are then determined on the basis of the above schedule and other items, so as to make equal said projected lengths of biting contact. Said vertical rolls 1 and 3 are housed in the vertical roll case 8. The difference in horizontal pressure between the vertical rolls 1 and 3 taking place during rolling does not produce bending moment, since the contact points  $Q_2$  and  $Q_5$  become parallel with each other. Therefore, the difference, if any, of reduction rates between the two flanges will not cause the rolled material to bend. Horizontal pressure acting on the vertical rolls 1 and 3 is, as follows:

$$P'_h = f B_h \sqrt{2 R' \Delta_h}$$

$$P_f = f B_f \sqrt{2 R \Delta_h}$$

Where:

$P'_h$ : horizontal pressure acting on the vertical roll 3 on the side of the head of the rail.

$P_f$ : horizontal pressure acting on the vertical roll 1 on the side of the base of the rail.

$R$ : diameter of the vertical roll 1.

$R'$ : diameter of the vertical roll 3

If  $B_h = B_f / 2.5$ , so  $\sqrt{2 R' \Delta_h} = \sqrt{2 R \Delta_h}$ ,

Therefore,  $P'_h < P_f$ .

The difference in horizontal pressure acting on the two vertical rolls due to the difference in reduction between the two flanges is absorbed by the contact of the part of the vertical roll to be subjected to smaller horizontal pressure with the horizontal roll. In this case, however, at the point of contact of the vertical roll with the horizontal roll, different peripheral speeds are produced, causing abrasion of the rolls, therefore, the following device will make the process more advantageous and is preferable. Sleeve rolls 11 are provided on the upper and lower parts of the vertical roll 3 of smaller diameter (on the side of the head of the rail) and held by bearings 13 and 14 set between said sleeve rolls and the axis 12 of the vertical roll, so that the sleeve rolls 11 contact the side of the horizontal rolls 4 and 4' and rotate independently of the vertical roll 3.

Then, by means of the vertical roll 1 on the side of the base of the rail which is subjected to greater horizontal pressure, the horizontal rolls 4 and 4' move toward the vertical roll 3 on the side of the head of the rail which is subjected to smaller horizontal pressure, causing the sleeve rolls 11 of the vertical roll 3 to contact the side of the horizontal rolls 4 and 4'. Therefore, the side of the vertical roll 3 which is subjected to smaller horizontal pressure, should be so made as to maintain the designed size at the time of contacting the horizontal rolls 4 and 4'. Thus, the horizontal rolls 4 and 4' move the vertical roll which is subjected to smaller horizontal pressure, and

therefore, accuracy of the size of every part of the product is maintained while allowing the horizontal rolls 4 and 4' to slip aside. However, this method is effective only during the first pass.

For more concrete understanding, the present invention is explained, as follows, using as an example, with mathematic formulas, the rolling of a prefigured steel piece having two flanges of the same thickness into a H-shaped steel product having flanges of a 1:3 ratio of thickness. The following is the definition of signs used in the explanation (See FIG. 4):

THICKNESSES OF FLANGES

| Pre-figured      | After 1st pass | After 2nd pass | After n'th pass | Product  |
|------------------|----------------|----------------|-----------------|----------|
| Thicker one..... | $T_{A0}$       | $T_{A1}$       | $T_{A2}$        | $T_{An}$ |
| Thinner one..... | $T_{W0}$       | $T_{W1}$       | $T_{W2}$        | $T_{Wn}$ |

REDUCTION RATE

|                  | At 1st pass | At 2nd pass | At n'th pass |
|------------------|-------------|-------------|--------------|
| Thicker one..... | $r_{A1}$    | $r_{A2}$    | $r_{An}$     |
| Thinner one..... | $r_{W1}$    | $r_{W2}$    | $r_{Wn}$     |

PROJECTED LENGTH OF BITING CONTACT

| $[\epsilon = \sqrt{2R\Delta T}]$ | $R = \text{Diameter of roll}$ | $\Delta T = \text{Reduction}$ |                 |
|----------------------------------|-------------------------------|-------------------------------|-----------------|
|                                  | At 1st pass                   | At 2nd pass                   | At n'th pass    |
| Thicker one.....                 | $\epsilon_{A1}$               | $\epsilon_{A2}$               | $\epsilon_{An}$ |
| Thinner one.....                 | $\epsilon_{W1}$               | $\epsilon_{W2}$               | $\epsilon_{Wn}$ |

Diameter of vertical roll

Thicker one:  $R_A$ ; Thinner one:  $R_W$   
Ratio of rolls in diameter:  $\alpha = R_A/R_W$

Reduction

$$\Delta T_n = T_{n-1} - T_n$$

Reduction rate

$$r_n = \Delta T_n / T_{n-1}$$

If so,

$$T_{Wn} = T_{W(n-1)} - \Delta T_{Wn} = T_{W(n-1)} - r_{Wn} T_{W(n-1)} = (1 - r_{Wn}) T_{W(n-1)}$$

In the same manner,

$$T_{An} = (1 - r_{An}) T_{A(n-1)}$$

Also,

$$r_{An} = \Delta T_{An} / T_{A(n-1)}$$

$$r_{Wn} = \Delta T_{Wn} / T_{W(n-1)}$$

$$\therefore r_{An} = r_{Wn} \frac{\Delta T_{An}}{\Delta T_{Wn}} = r_{Wn} \frac{T_{W(n-1)}}{T_{A(n-1)}} = \frac{r_{Wn}}{\alpha_n} \frac{T_{W(n-1)}}{T_{A(n-1)}}$$

$$T_{An} = \left(1 - \frac{r_{Wn}}{\alpha_n} \frac{T_{W(n-1)}}{T_{A(n-1)}}\right) T_{A(n-1)} = T_{A(n-1)} - \frac{r_{Wn}}{\alpha_n} T_{W(n-1)}$$

$$\epsilon_{A1} = \sqrt{2R_A \Delta T_{A1}}, \epsilon_{W1} = \sqrt{2R_W \Delta T_{W1}}$$

Since

$$\epsilon_{A1} = \epsilon_{W1}, \text{ so } R_A \Delta T_{A1} = R_W \Delta T_{W1}$$

$$\therefore \Delta T_{W1} / \Delta T_{A1} = R_A / R_W = \alpha$$

This means that if the proportion of reduction is reverse to the proportion of diameters of vertical rolls, the projected lengths of biting contact of the rolls become equal.

Also,

$$T_{A1} = T_{A0} - \Delta T_{A1} = T_{A0} - r_{A1} T_{A0} = (1 - r_{A1}) T_{A0}$$

(b<sub>1</sub>)

In the same manner,

$$T_{W1} = T_{W0} - \Delta T_{W1} = T_{W0} - r_{W1} T_{W0} = (1 - r_{W1}) T_{W0}$$

(c<sub>1</sub>)

At the 2nd pass,

$$T_{W2} = T_{W1} - \Delta T_{W2} = (1 - r_{W2}) T_{W1} = (1 - r_{Wn}) (1 - r_{W1}) T_{W0}$$

75

However, if the ratios (a) of the diameters of the rolls are the same for all the passes; and  $r_{W2} \rightarrow r_{W1} \rightarrow r_W$

$$T_{W2} = (1 - r_W)^2 T_{W0} \quad (c_2)$$

$$5 \quad T_{A2} = T_{A1} - \frac{r_W}{\alpha} T_{W1} = (1 - r_{A1}) T_{A0} - \frac{r_W}{\alpha} (1 - r_W) T_{W0} \quad (b_2)$$

In the same manner, at the 3rd pass,

$$T_{W3} = (1 - r_W)^3 T_{W0} \quad (c_3)$$

$$10 \quad T_{A3} = T_{A2} - \frac{r_W}{\alpha} T_{W2} = (1 - r_{A1}) T_{A0} - \frac{r_W}{\alpha} (1 - r_W) T_{W0} - \frac{r_W}{\alpha} (1 - r_W)^2 T_{W0}$$

$$15 \quad = (1 - r_{A1}) T_{A0} - \frac{r_W}{\alpha} \left\{ (-r_W) + (1 - r_W)^2 \right\} T_{W0} \quad (b_3)$$

$$20 \quad \text{Therefore, at the } n^{\text{th}} \text{ pass,} \quad T_{Wn} = (1 - r_W)^n T_{W0} \quad (c_n)$$

$$25 \quad T_{An} = (1 - r_{A1}) T_{A0} - \frac{r_W}{\alpha} \left\{ (1 - r_W) + (1 - r_W)^2 \right. \\ \left. + \dots (1 - r_W)^{n-1} T_{W0} = (1 - r_{A1}) T_{A0} - \frac{1}{\alpha} \{ (1 - r_W) - (1 - r_W)^n \} T_{W0} \right. \quad (b_n)$$

30 Assuming that,

$$T_{A0} = T_{W0} = T_0$$

$$r_{A1} = \frac{r_W}{\alpha} \frac{T_{W0}}{T_{A0}} = \frac{r_W}{\alpha}$$

$$35 \quad \therefore T_{Wn} = (1 - r_W)^n T_0 \quad (c)$$

$$T_{An} = \left(1 - \frac{r_W}{\alpha}\right) T_0 - \frac{1}{\alpha} [1 - r_W] - (1 - r_W)^n T_0$$

$$40 \quad = \left[ \left(1 - \frac{1}{\alpha}\right) + \frac{1}{\alpha} (1 - r_W)^n \right] T_0 \quad (b)$$

In case actual figures are introduced into the formula (b), as follows:

45 For rolling a prefigured steel piece having flanges of the same thickness into a H-shaped steel product having flanges of a ratio of 1:3 of thickness, during which rolling the reduction rates at each pass are 0.1 and 0.15 respectively for the thicker flange and the thinner flange, the required number of passes 50 is:

Since  $r_W = 0.15, r_A = 0.10$  and  $T_{A0} = T_{W0}$

$$\alpha = \frac{0.15}{0.10} = 1.5$$

$$3(1 - 0.15)^n = \left(1 - \frac{1}{1.5}\right) + \frac{1}{1.5} (1 - 0.15)^n$$

$$3 \times 0.85^n = \left(1 - \frac{1}{1.5}\right) + \frac{1}{1.5} \times 0.85^n$$

$$4.5 \times 0.85^n = 0.5 + 0.85^n$$

$$n \log 0.85 = \log 0.142857$$

$$n = \frac{0.845}{0.0706} = 12$$

That is, the desired product will be obtained at the 12th pass.

However, in actual case where the thicknesses of flanges of the prefigured steel piece, those of the desired product, the diameter of either roll and the reduction rate of each roll are already known, the diameter of the other roll can be easily obtained from the reverse proportion of reduction rates. As mentioned above, the present invention makes it possible to greatly stabilize rolling operations for the production of H-

shaped steel products having flanges of different thicknesses and similarly shaped steel products, by equalizing the projected lengths of biting contact of the two rolls on the rolled material, thereby eliminating bend and torsion of the rolled material caused by horizontal pressure.

However, in addition to the above relationship, successful rolling can be attained also by making nearly equal the projected lengths of biting contact of the rolls by making the diameter of the roll which is subjected to the greater reduction rate, smaller than that of the other roll. In other words, when producing products having flanges of different thicknesses from a material piece having flanges of the same thickness, it is natural that the difference in stretching rate should occur at every pass. However, even in the ordinary type of rolling for 15 the production of H-shaped steel products having flanges of the same thickness, these flanges are not always the same in stretching rate. This is due mostly to play of parts of the rolling mill or difficulty in obtaining rolled materials of a desired size.

The present invention makes it possible to produce 20 products having flanges of different desired thicknesses by taking up the greatest difference of allowance of stretching rate between the two flanges and by carrying out the rolling operation several times taking into consideration the difference of allowance of stretching rate between the flanges for 25 each rolling operation.

What I claim is:

1. In the rolling of steel material with the universal rolling

mill, which includes a pair of vertical rolls and a pair of horizontal rolls, into asymmetrical H-shaped products having flanges of different thicknesses and similarly shaped products, the improvement comprising the steps of providing one of said pair of vertical rolls with a smaller diameter than the other, and causing said pair of vertical rolls to contact said steel material such that a line connecting the initial points of contact of said vertical rolls with said material is parallel to a line connecting the centers of said vertical rolls, thereby causing the projected lengths of biting contact of said vertical rolls with said material to be equal.

2. In a universal rolling mill for making asymmetrical H-shaped products having flanges of different thicknesses and similarly shaped products, said mill comprising a pair of horizontal rolls and a pair of vertical rolls, said vertical rolls positioned to roll said flanges, the improvement wherein the diameter of one of said vertical rolls is smaller than that of the other, such difference in diameter corresponding to the difference in thickness of said flanges, and comprising a pair of sleeve rolls mounted on said one of said vertical rolls having the smaller diameter, said pair of sleeve rolls contacting said horizontal rolls.

3. In a universal rolling mill as claimed in claim 2, wherein said sleeve rolls are mounted around the axis at the upper and lower parts of said vertical roll having the smaller diameter, said small diameter vertical roll and said sleeve rolls being mounted to rotate independently.

30

35

40

45

50

55

60

65

70

75